

Dec. 19, 1933.

F. C. KELLEY

1,940,308

METHOD OF MAKING CARBIDES

Filed Sept. 26, 1928



Inventor:  
Floyd C. Kelley,  
by *Charles E. Tullar*  
His Attorney.

## UNITED STATES PATENT OFFICE

1,940,308

## METHOD OF MAKING CARBIDES

Floyd C. Kelley, Schenectady, N. Y., assignor to  
General Electric Company, a corporation of  
New York

Application September 26, 1928  
Serial No. 308,565

11 Claims. (CL 23—208)

The present application which is a continuation-in-part of my co-pending application Serial No. 245,267, filed Jan. 7, 1928, matured to Patent No. 1,794,300 dated Feb. 24, 1931, and entitled 5 Hard metal compositions, relates to a method of heat treating materials, containing an appreciable quantity of carbon, without affecting the carbon content thereof and more particularly to a method of making carbides so that they will 10 have a definite carbon content.

In making hard metal compositions, such as disclosed in the patent to Schröter No. 1,549,615, which consist largely of a carbide of a metal of the tungsten group but contain an appreciable 15 quantity of auxiliary metal of lower melting point than the carbide, for example cobalt, it is desirable to provide a product of uniform quality. This can be accomplished only by controlling accurately the quantities of the various constituents 20 entering into the composition. While it is an easy matter to control the tungsten and cobalt content of such compositions, it is difficult to control accurately the carbon content of the carbide by methods heretofore employed.

25 It is preferable in the manufacture of tungsten carbide which is to be employed in the manufacture of hard metal compositions, such as described in the Schröter patent, to combine from 5.5% to 6.2% of carbon with the tungsten. In 30 making the carbide, it has been customary to effect the carbonization of the tungsten by means of powdered carbon placed with the tungsten in an open carbon furnace, an excess amount of powdered carbon being placed in the carbon holder. During the carbonization process, a certain 35 amount of powdered carbon is burned out. However, it is difficult to determine when the proper amount of carbon has been removed and as a result the carbide often contains less than 5.5% 40 or more than 6.2% of carbon.

In carrying out the present invention, the tungsten and carbon in powdered form and in definite proportions are placed in a closed carbon receptacle and the receptacle is heated in a hydrogen 45 atmosphere to a relatively high temperature and for a period of time long enough to cause combination of the tungsten and carbon. Under these conditions, the quantity of carbon in the finished product is found to be the exact amount 50 placed in the carbon receptacle with the tungsten. Tools, dies and other materials made from such a product are of unvarying quality.

The novel features which I believe to be characteristic of my invention are set forth with particularity in the appended claims. The invention

itself, however, will best be understood from reference to the following specification when considered in connection with the accompanying drawing, in which the single figure shows partly in elevation and partly in section, an electric furnace 60 whereby my invention may be carried into effect.

Referring more particularly to the drawing, I have indicated at 10 an electric furnace comprising a steel casing 11 and a concentric coaxial alumina tube 12, the latter being surrounded by 65 a molybdenum heating coil 13 connected at its ends to binding posts 14 and 15 which may be connected to a suitable source of energy, not shown. The space between the casing 11 and the outer surface of the tube 12 is filled with 70 suitable insulating material such as powdered alumina 16.

Hydrogen is supplied to the interior of the casing 11 through inlet pipes 17 and 18 so that the molybdenum heating coil and the outer surface of tube 12 are completely surrounded at all times by an atmosphere of hydrogen. Tube 12 permits the passage of hydrogen therethrough. Hydrogen is also supplied at one end of the tube 12 from a pipe 19 and through valve 20. The 80 hydrogen flows through the tube 12 to the opposite end thereof where it is burned as indicated at 21. A water jacketed chamber 22, having inlet and outlet water pipes 23 and 24, respectively, is secured to one end of the furnace 85 for a purpose which will be disclosed presently.

In carrying the invention into effect, tungsten and carbon in powdered form and in the desired proportions, that is, about 94% tungsten and about 6% carbon are placed in a carbon receptacle 25 which is closed by a carbon plug 26. The receptacle 25 is placed in the furnace 10 and heating current is supplied to the coil 13 while hydrogen is caused to flow over and around the receptacle 25. The powdered materials are 90 heated in this manner at a temperature above 1000° C. but below the melting point of the tungsten, for example about 1500° C. for about three hours, at the end of which time the tungsten is substantially completely carbonized and substantially no free carbon powder remains in receptacle 25. At the end of the three hour period, the circuit to coil 13 is opened, the hydrogen supply shut off and the carbon receptacle pushed in the water jacketed chamber 22 where it is 95 allowed to cool to room temperature. Thereafter a plug 27 may be removed from the water jacketed chamber and the receptacle 25 removed therefrom.

When carbonized in the manner shown, it 110

will be found that although the receptacle 25 is made of carbon, substantially none of it combines with the tungsten powder and that the percentage of powdered carbon placed in the receptacle originally does not vary more than one tenth of one per cent from the carbon content of the finished product. Although I find it advantageous to heat the powdered material to a temperature of 1500° C. for about three hours, 10 a lower temperature may be employed if desired, although the heating period would be lengthened under such circumstances. Likewise the temperature may be raised above 1500° C. and the heating period shortened somewhat.

15 My explanation of the above action is that the hydrogen in passing through the carbon receptacle 25 combines with a certain portion of the carbon thereof to form a hydro-carbon gas. When this hydrocarbon gas comes in contact with the tungsten metal a combination between the carbon in the gas and the tungsten metal occurs, tungsten carbide being formed while hydrogen is liberated. The liberated free hydrogen in the tube being in a very active condition, combines 20 with the powdered carbon of the charge to reform the hydrocarbon gas. The hydrocarbon gas in the tube therefore remains in a condition of equilibrium with respect to the carbon at the temperature employed while effecting carburization of the tungsten. The reactions which take 25 place may be indicated as follows:



30 Hence  $mC + mW \rightarrow mWC$  and  $nH + mC$  (in charge)  $\rightarrow C_mH_n$  etc.

until all tungsten has been carburized.

While I have shown the use of a carbon receptacle, other porous receptacles containing an appreciable amount of carbon in their composition may be employed if desired. While such receptacles should permit diffusion of hydrogen therethrough, they should not permit diffusion 45 at such a rate that any hydrogen passing through the receptacle is uncombined with carbon.

Although I have illustrated my invention in connection with the formation of tungsten carbide, it is by no means limited to the formation 50 of carbide or to this particular carbide. For example, the invention may be applied to material, such as iron or steel which contains an appreciable amount of carbon, when it is desired to anneal such material without decarbonization. If such 55 material is enclosed in a wrought iron pipe receptacle provided with closed pipe caps and then heated to an annealing temperature in a hydrogen furnace, it is found that the carbon content of the annealed metal is unchanged by the process. The container in such a case should have 60 enough carbon in its composition to combine with all the hydrogen which penetrates to the interior of the receptacle and walls should be thick enough so that the walls are never completely decarbonized during the annealing period.

What I claim as new and desire to secure by Letters Patent of the United States, is:—

1. The method of heat treating solid material containing an appreciable quantity of carbon so 70 as to prevent variation of the carbon content thereof, which comprises placing in a furnace a closed receptacle containing said material, the walls of said receptacle containing an appreciable quantity of carbon and being porous to 75 hydrogen, and heating the receptacle in said fur-

nace at an elevated temperature but below the melting point of said material, and in a hydrogen atmosphere.

2. The method of forming a carbide of a metal 80 which comprises placing the metal and carbon, each in powdered condition, in a closed receptacle, the walls of which are porous to hydrogen and contain an appreciable quantity of carbon, and heating said receptacle in a current of hydrogen at an elevated temperature but below the melting point of said metal for a period of time long enough to cause combination of the powdered carbon and metal.

3. The method of forming a carbide with an element of the tungsten group, which comprises 90 heating said element and carbon in powdered form at an elevated temperature below the melting point of said element and in a closed carbon receptacle while said receptacle is surrounded by an atmosphere of hydrogen.

4. The method of forming tungsten carbide which comprises placing about 93.8% to 94.5% tungsten powder and about 6.2% to 5.5% carbon powder in a carbon receptacle, closing said receptacle and heating it to a temperature of about 100 1500° C. for about three hours in hydrogen.

5. The method of forming tungsten carbide which comprises placing approximately 94% tungsten powder and approximately 6% carbon powder in a carbon receptacle, closing said receptacle and heating it for an appreciable period of time in an atmosphere of hydrogen at a temperature above 1000° C. but below the melting point of tungsten.

6. The method of forming a carbide of an element of the tungsten group which comprises placing approximately 94% of said element in powdered form and 6% of carbon in powdered form in a receptacle, the walls of which consist mainly of carbon, closing said receptacle and 115 heating it for an appreciable period of time in an atmosphere of hydrogen at a temperature above 1000° C. but below the melting point of said element.

7. The method of forming a carbide of an 120 element of the tungsten group which comprises placing approximately 94% of said element in powdered form and approximately 6% of carbon in powdered form in a receptacle and heating the powdered mixture at an elevated temperature 125 but below the melting point of said element and in the presence of a hydro-carbon gas which at that temperature is in a state of equilibrium with respect to carbon.

8. The method of forming a carbide of a metal 130 which comprises placing a powdered composition comprising said metal and carbon in a closed carbon tube and heating said closed tube in hydrogen at a relatively high temperature but below the melting point of said metal and for a 135 period of time sufficient to cause combination of said metal and powdered carbon.

9. The method of forming a carbide of a metal which comprises placing a powdered composition 140 consisting substantially of said metal and carbon in a closed carbon tube, the quantity of powdered carbon being sufficient to convert substantially all of said metal to a carbide of said metal and heating said closed tube in a hydrogen atmosphere at an elevated temperature but below the melting point of said metal and for a 145 period of time sufficient to cause combination of said metal with said carbon.

10. The method of forming a carbide of a metal which comprises placing in a furnace a closed 150

- carbon tube containing a mixture consisting mainly of said metal but containing carbon only in sufficient quantity to convert substantially all of said metal to a carbide of said metal and heating said tube in a hydrogen atmosphere at a temperature above 1000° C. but below the melting point of said metal for a period of time sufficient to convert said metal to a carbide of said metal.
- 5 11. The method of forming a carbide of a metal which comprises placing in a furnace a closed carbon tube containing a powdered mixture consisting mainly of said metal and carbon, said carbon being present in such quantity that when combined with said metal substantially no free carbon will be present in said tube and heating 80 said closed tube in a hydrogen atmosphere at a temperature above 1000° C. but below the melting point of said metal for a period of time sufficient to cause combination of said metal and carbon.
- 10 11. The method of forming a carbide of a metal which comprises placing in a furnace a closed

FLOYD C. KELLEY. 85

15 90

20 95

25 100

30 105

35 110

40 115

45 120

50 125

55 130

60 135

65 140

70 145

75 150